

# UNITED STATES PATENT OFFICE.

SAMUEL B. FIELD, OF HOLBROOK, MASSACHUSETTS, ASSIGNOR TO PNEUMATIC SCALE CORPORATION, LIMITED, OF QUINCY, MASSACHUSETTS, A CORPORATION OF MAINE.

## MOISTURE-PROOF ADHESIVE COMPOUND.

1,307,247.

Specification of Letters Patent. Patented June 17, 1919.

No Drawing.

Application filed December 20, 1917. Serial No. 208,074.

*To all whom it may concern:*

Be it known that I, SAMUEL B. FIELD, a citizen of the United States, residing at Holbrook, county of Norfolk, State of Massachusetts, have invented a certain new and useful Improvement in Moisture-Proof Adhesive Compound, of which the following is a specification, reference being had therein to the accompanying drawings.

10 The object of the invention is to provide a moisture proof adhesive compound which in normal atmospheric conditions is hard, cohesive and non-sticky, and which when heated to a temperature considerably above 15 any normal atmospheric temperature becomes sticky. The special use to which the said invention is intended to be applied is to provide an adhesive moisture proof coating for packages in which package goods 20 are put up and in which the material of the shell itself or of the wrapper is of non-moisture proof material. It is important that this coating shall not only be moisture proof and adhesive and non-sticky when 25 dry, but also it is preferable that it should be pliable and tough when dry so that it will not readily crack when the paper to which it is applied is bent.

The invention will be fully understood 30 from the following description and the novel features thereof will be pointed out and clearly defined in the claims at the close of this specification.

The base of the composition is resinous 35 pitch, preferably Burgundy pitch because the melting point is considerably lower than other kinds of pitch. The pitch is combined with paraffin and rosin oil, preferably in about the following proportions, one and 40 one-half pounds of pitch, three ounces of paraffin and eight one-hundredths of an ounce of rosin oil. In preparing the composition the pitch is melted and then the paraffin and rosin oil are added, the ingredients 45 all being thoroughly mixed together while in a highly heated condition. It may then be allowed to cool and form a solid mass which is dry under normal atmospheric conditions and non-sticky. When it is desired 50 to apply a coating of said composition to any surface the composition is again heated to a high degree sufficient to bring it to a liquid or semi-liquid state and then a thin film is spread over the surface of the 55 article which is desired to be rendered mois-

ture proof. As soon as the film which has been spread on the said surface cools to the normal atmospheric temperature, it hardens but is sufficiently pliable so that if it has been spread on a sheet of paper the sheet of 60 paper may be bent, as in wrapping up a package, without cracking. If it is then desired to cause an adhesion between the sheet of paper on which said coating has been spread and the package about which 65 the sheet is to be wrapped or to cause an adhesion between the coated sheet and another sheet of paper the two sheets of paper which are to be given adhesive connection are superimposed one upon the other, or in 70 the case of a package the coated sheet may be wrapped around the package, and then heat is applied to the outer surface sufficient to melt the adhesive coating so as to render 75 it sticky. By applying pressure while the coating is sticky the two surfaces will be caused to adhere together. The two articles which are to be united are then allowed to cool and the adhesive coating will become 80 dry and firmly unite together the two articles or surfaces.

The paraffin and rosin oil both aid in making the film pliable. If the rosin oil or some equivalent thereof is omitted and paraffin alone is mixed with the pitch, so much paraffin has to be used that the compound is not sticky enough when hot to give the proper adhesive quality. If the paraffin or some equivalent thereof is not used and if 85 rosin oil alone is used with the pitch to render it pliable so much rosin oil has to be used to make the film pliable that the mixture is non-drying when cool and the coated sheet will also be sticky in normal temperature. The use of both paraffin and rosin oil 90 keeps the coating or the film in proper condition so that although it is sticky when hot, it is both pliable and non-sticky when cool or when it is at any normal atmospheric 95 temperature.

100 What I claim is:

1. A moisture repellent adhesive compound consisting of a composition of pitch, paraffin and rosin oil characterized by being dry and non-sticky under normal atmospheric conditions and of becoming soft and sticky when heated to a high degree of temperature and capable of adhesively uniting two surfaces together and again becoming dry and non-sticky and capable of retaining 105 110.

two surfaces adhesively united when it is cooled again to normal temperature.

2. A moisture repellent adhesive compound consisting of a composition of Bur-  
5 gundy pitch, paraffin and rosin oil char-  
acterized by being dry and non-sticky under  
normal atmospheric conditions and of be-  
coming soft and sticky when heated to a  
10 high degree of temperature and capable of  
adhesively uniting two surfaces together and  
again becoming dry and non-sticky and ca-  
pable of retaining two surfaces adhesively  
united when it is cooled again to normal  
temperature.

15 3. A moisture repellent adhesive com-  
pound consisting of a composition of pitch,  
paraffin and rosin oil in substantially the  
following proportions, one and one-half  
20 pounds of pitch, three ounces of paraffin,  
and eight one-hundredths of an ounce of  
rosin oil, said composition being character-  
ized by being dry and non-sticky under nor-  
mal atmospheric conditions and of becom-

ing soft and sticky when heated to a high  
degree of temperature and capable of ad-  
hesively uniting two surfaces together and  
again becoming dry and non-sticky and ca-  
pable of retaining two surfaces adhesively  
united when it is cooled again to normal  
temperature.

30 4. A moisture repellent adhesive com-  
pound consisting exclusively of pitch, par-  
affin and rosin oil thoroughly mixed to-  
gether, said ingredients being compounded  
in substantially the following proportions, 35  
one and one-half pounds of pitch, three  
ounces of paraffin and eight one-hundredths  
of an ounce of rosin oil, said composition  
being sticky and capable of adhesively unit-  
ing two surfaces together when the composi-  
40 tion is softened by a high degree of heat,  
and being dry and non-sticky when cooled  
to normal atmospheric temperature.

In testimony whereof I affix my signature.

SAMUEL B. FIELD.